

## UNITED STATES PATENT OFFICE

2,222,783

## SPINNING

Robert Pierce Roberts and Robert McVane Dingley, Spondon, near Derby, England, assignors to Celanese Corporation of America, a corporation of Delaware

No Drawing. Application September 9, 1937, Serial No. 163,095. In Great Britain September 23, 1936

5 Claims. (Cl. 18—54)

This invention relates to the spinning of rubber threads from aqueous dispersions of rubber.

We have found that a very satisfactory spinning solution for the production of rubber threads by extrusion into a suitable acid bath, can be made by mixing an aqueous dispersion of rubber such as rubber latex with a dispersion containing zinc oxide, sulphur, one or more vulcanisation accelerators and a dispersing agent in amount sufficient to impart to the spinning solution a viscosity between about 135 and 165 on a scale in which the viscosity of a 70% solution of glycerine measured at 25° C. is 100. By a 70% aqueous solution of glycerine is meant a solution produced by diluting 70 volumes of glycerine with 30 volumes of water.

We have found that the viscosity of the spinning solution is of very great importance and that unless the viscosity lies within the limits specified above instability in spinning and/or weakness in the resulting thread is apt to result. One of the most important factors effecting the viscosity of the spinning solution is the nature and amount of the dispersing agent used. We have found that the casein is particularly suitable as a dispersing agent for the purpose of the invention and is much superior for this purpose to dispersing agents such as gelatine, glue, viscose and soaps, for example the sodium, zinc or calcium salts of stearic, oleic, palmitic and similar higher fatty acids. The amount of casein used should be strictly controlled to give the desired viscosity. We have found proportions of 0.05 to 0.5%, e. g. 0.1, 0.2, or 0.3% of casein on the weight of the rubber, to be suitable.

The selection of a suitable accelerator is also important. We have found that it is of particular advantage to use a mixture of two or more accelerators, one being of the mercaptan class, e. g. mercaptobenzthiazole, and the other of the guanidine class, for example diphenyl guanidine. Accelerators such as mercaptobenzthiazole alone tend to coagulate the spinning solution. On the other hand accelerators such as diphenyl guanidine act too slowly to be used alone. Mixtures containing a member of each of these classes, however, ensure rapid vulcanisation without a danger of premature coagulation of the spinning solution. Thus the spinning solution may contain for example a proportion ranging from 0.25

to 2%, e. g. 0.5 to 1%, of such a mixture, e. g. a mixture of mercaptobenzthiazole and diphenyl guanidine in the ratio of about two to one, on the weight of the rubber. Other classes of accelerators, for example the xanthates such as sodium isopropyl xanthate, dithio acids, for instance sodium and zinc diethyl-thiocarbamates, and the thiuram sulphides, for instance tetraethylthiuram-disulphide, are less suitable.

The spinning solution may contain in addition to the zinc oxide other white or coloured pigments. A very suitable white pigment for use is titanium oxide. When organic colouring agents are used care should be taken that these are stable towards sulphur.

The spinning solution may also contain an antioxidant such for example as the substance sold as "Nonox S."

Spinning is preferably effected by extruding the solution into a coagulating bath comprising an aqueous solution of acetic acid, for example a 15-25% solution containing 15-25% of acetic acid. Other dilute acids, however, can be used, for example hydrochloric acid of similar pH value. After leaving the coagulating bath the thread is preferably drawn first through a washing bath which may contain for example 10-20% of ammonium carbonate or other mildly alkaline substance in suitable concentration to neutralise the acidity resulting from the coagulating bath, and then through a bath containing a lubricant such as a textile soap adapted to prevent sticking of the threads during subsequent operations. A 5-15% aqueous solution of a textile soap has been found suitable for this purpose. The use of such a lubricating bath has been found preferable to the use for the same purpose of solid substances such as French chalk or graphite. After leaving the lubricating bath the thread may be collected by suitable means and vulcanised in package form. We prefer to collect the thread on a collapsible swift and to remove the thread therefrom after drying and vulcanise it in hank form. Other methods of collection may, however, be used, for instance the thread may be deposited in loose coils in a suitable container and dried and vulcanised before winding. The coils may be formed for example by reciprocating the container and the thread guide at right angles at different speeds. Or centrifugal methods of col-

lection may be used. Drying and vulcanising the thread continuously with its production is difficult on account of the time required for vulcanisation unless very rapid accelerators are used, in which case there is some danger of premature coagulation.

The following example illustrates the invention:

*Example*

10 Rubber latex containing about 60% rubber and having a viscosity of about 230 on a scale in which the viscosity of a 70% aqueous solution of glycerine is 100 measured at 25° C., is compounded with the following components, the percentages being on the weight of dry rubber in the latex:

|                | Per cent |
|----------------|----------|
| Titanium oxide | 6        |
| Zinc oxide     | 4        |
| Sulphur        | 3        |
| Accelerator    | 0.5      |
| Anti-ager      | 1        |
| Casein         | 0.2      |

25 (The accelerator consists of a mixture of mercaptobenzthiazole and diphenyl guanidine in the ratio of about 2:1).

These components are ground together in a small amount of water to a particle size of 1-2  $\mu$  30 and added to the latex. If insufficient water has been used in the grinding to bring the viscosity of the final dispersion containing the latex to 165 further water is added until the viscosity is 35 between 165 and 135 on the scale referred to above.

The resulting dispersion is spun into a 20% aqueous acetic acid bath at such a speed that the time of immersion is 9-10 seconds. The resulting threads are carried through a washing 40 bath consisting of a 15% aqueous solution of ammonium carbonate, then through an aqueous bath containing 10% of textile soap and are collected on collapsible swifts and dried thereon for several hours at between 60-70° C.

45 The products are then removed from the swift and vulcanised in hank form for about 36 hours at between 70 and 90° C.

Having described our invention what we desire to secure by Letters Patent is:

50 1. Process for the production of rubber filaments, threads and like products which comprises spinning into an aqueous solution of acetic acid of from 15 to 25% strength, an aqueous

dispersion of rubber having a kinematic viscosity ranging from about 1.35 to about 1.65 times that of a 70% aqueous solution of glycerine measured at 25° C., said dispersion containing casein as a dispersing agent, and collecting the 5 formed products.

2. Process for the production of rubber filaments, threads and like products which comprises spinning into an aqueous solution of acetic acid of about 20% strength, an aqueous dispersion of rubber having a kinematic viscosity ranging from about 1.35 to about 1.65 times that of a 70% aqueous solution of glycerine measured at 25° C., said dispersion containing from 0.1 to 0.3% on the rubber content of the 10 casein as a dispersing agent together with zinc oxide, sulphur and from 0.25 to 2% on the rubber content of a mixture of mercapto-benzthiazole and diphenyl guanidine in the ratio of about 2:1, the time of immersion in the bath being 20 between 9 and 10 seconds, carrying the products through an aqueous solution of a mild alkali, then through an aqueous soap bath, collecting them, drying them and vulcanizing them. 25

3. A spinning solution for use in the production of rubber filaments, threads and like products, comprising an aqueous dispersion of rubber having a kinematic viscosity ranging from about 1.35 to about 1.65 times that of a 70% aqueous 30 solution of glycerine measured at 25° C.

4. A spinning solution for use in the production of rubber filaments, threads and like products, comprising an aqueous dispersion of rubber having a kinematic viscosity ranging from about 35 1.35 to about 1.65 times that of a 70% aqueous solution of glycerine measured at 25° C., said dispersion containing casein as a dispersing agent.

40 5. A spinning solution for use in the production of rubber filaments, threads and like products, comprising an aqueous dispersion of rubber having a kinematic viscosity ranging from about 1.35 to about 1.65 times that of a 70% aqueous solution of glycerine measured at 25° 45 C., said dispersion containing from 0.05 to 0.5% on the rubber content of casein as a dispersing agent together with zinc oxide, sulphur and a mixture of vulcanization accelerators, at least one being of the mercaptan class and at least 50 another of the guanidine class.

ROBERT PIERCE ROBERTS.  
ROBERT McVANE DINGLEY.